# EUROPEAN PATENT SPECIFICATION

(11) **EP 0 066 176 B1**
(45) Date of publication and mention of the grant of the patent: **09.01.1985**
(21) Application number: 82104326.2
(22) Date of filing: 17.05.1982
(51) Int. Cl.: B41N 3/08

(54) **Fountain solutions suitable for use in lithographic offset printing**
Feuchtwasser für lithographische Offsetdruckverfahren
Solutions de mouillage pour impression lithographique offset

(30) Priority: 18.05.1981 US 264076
(43) Date of publication of application: 08.12.1982
(73) Proprietor: UNION CARBIDE CORPORATION, Danbury Connecticut 06817 (US)
(72) Inventor: Burns, Richard Jude, Piscataway (08854) (US); Willeboordse, Friso George, Warren New Jersey (US); Cohen, Martin Frank, Yorktown Heights New York 10598 (US)
(74) Representative: Barz, Peter, Dr.

## Description

This invention is directed to an improved fountain solution suitable for use in a lithographic offset printing press, which solution contains a mixture of a polyol and/or glycol ether partially soluble in water and a polyol and/or glycol ether completely soluble in water.

Lithographic printing operations require the use of a dampening or fountain solution to achieve proper operation of the press so that good quality prints are obtained.

The fountain solution is generally a blend or mixture of water, acids, salts, solvents, and naturally occurring polymeric materials, such as gum arabic, and/or a variety of synthetic polymers. The purpose of the fountain solution is to wet the non-image areas of a printing plate and thus prevent ink from depositing in these non-image areas. Should the ink deposit in the non-image area, a poor quality print results. Traditionally, alcohols, especially isopropanol, were used in fountain solutions up to 30 percent volume concentration levels to achieve best performance in operation of the press with attendant high quality prints. The basis for using isopropyl alcohol resides partly in its ability to transport the fountain solution to the printing plate by means of the inked rollers in the press or through its own roller train. This property has been attributed to the low surface tension of the aqueous solution containing the isopropyl alcohol. This allows the fountain solution to wet and mix with the ink in the Dahlgren system or to keep ink and fountain solution separate as in lithographic presses with conventional dispersing systems. However, when the fountain solution is transported by the rollers in the form of a thin film, volatile components, especially the alcohol, are lost. Aside from the cost considerations in losing the alcohol by evaporation, safety considerations urge against its use. Thus, it is desirable to find a substitute for the volatile alchol which does not have the problems associated with using isopropyl alcohol.

U.S. Patent 3,877,372 describes an attempt to eliminate isopropanol from the fountain solution and use a mixture of butyl cellosolve, a silicone glycol copolymer, and a defoamer.

A commerically available fountain solution utilizes 2-ethyl-1,3-hexanediol as a replacement for isopropyl alcohol to provide an isopropyl alcohol free fountain solution. The use of 2-ethyl-1,3-hexanediol eliminates the toxic and flammable properties associated with isopropyl alcohol containing fountain solutions. Also, fountain solutions containing the 2-ethyl-1,3-hexanediol provide a high quality printed product on a lithographic press.

However, it has been found that in using the 2-ethyl-1,3-hexanediol containing fountain solutions, the appearance of tinting and/or banding in the print is observed in many instances. Tinting is the deposition of minute ink droplets in the non-image area of the print resulting in the appearance of a light tint. Banding is the appearance of narrow dark streaks in the print. Thus, there is a desire to develop a non-isopropyl alcohol containing fountain solution whose use would substantially eliminate the appearance of tinting and/or banding in a print.

It has now been found that when a mixture of a polyol and/or glycol ether partially soluble in water and a polyol and/or glycol ether completely soluble in water is used in a fountain solution, tinting and/or banding in the resulting print is substantially reduced and in many instances eliminated.

The use of such a mixture as a replacement for isopropyl alcohol eliminates the toxic and flammable properties of conventional isopropyl alcohol-containing fountain solutions and provides a fountain solution that has the other desirable properties which provide a high quality printed product on a lithographic plate.

The fountain solution contains between about 0.5 and about 10 percent by volume of the mixture.

The mixture of polyols and/or glycol ethers which is suitable for use in this invention includes a polyol and/or glycol ether which is partially soluble in water, such as 2-ethyl-1 ,3-hexanediol, Esterdiol-204, i.e., Hexyl Cellosolve, i.e., Hexyl Carbitol, i.e., and the like, and a polyol and/or glycol ether which is completely soluble in water, such as propylene glycol, ethylene glycol, dipropylene glycol, diethylene glycol, hexylene glycol, triethylene glycol, tetraethylene glycol, tripropylene glycol and 1,5-pentanediol.

The fountain solutions are preferably used as aqueous acidic solutions. Phosphoric acid is a preferred acid for use in acidifying the formulation. Other acids which can be used include inorganic as well as organic acids, such as acetic acid, nitric acid, hydrochloric acid, and the like. A buffering agent, such as ammonium acetate can also be included.

The fountain solution is generally maintained at a pH of from about 2 to about 5. However, the particular pH at which a given solution will be maintained will depend upon factors, such as the type of water-soluble polymer used, other ingredients in the solution as well as the type of substrate employed in the lithographic printing plate, and the like.

Other additives which may be used in the fountain solution include preservatives such as phenol, sodium salicylate, and the like; corrosion inhibitors such as ammonium bichromate, magnesium nitrate, zinc nitrate, and the like; hardeners such as chromium alum, and the like; organic solvents such as cyclic ethers, e.g., 4-butyrolactone, and the like; low molecular weight aldehydes, such as formaldehyde, glutaraldehyde, and the like. These additives are generally used in amounts of from about 0.1 to about 10 percent by volume.

### EXAMPLES

The following examples serve to illustrate specific embodiments of this invention and it is not intended that the invention shall be limited by the examples.

### Control

The following ingredients were mixed together to form a fountain solution base:
14.17 g (0.5 ounce) gum arabic
14.17 g (0.5 ounce) phosphoric acid (a 5% solution in water), and
3600 g (127.0 ounce) water

To the formulation, which equalled one gallon (3629 g) (128 ounces) was added 36.85 g (1.3 ounces) of 2-ethyl-1,3-hexane-diol to make a 1 volume percent concentration of 2-ethyl-1,3-hexanediol.

The fountain solution was used on a 63.5 cm (25 inch) production size press with Dahlgren recirculating dampening system. The press was run with the damper set at speeds of 40, 50 and 60 running approximately 200 sheets of paper at each setting. The optical density of sheets was measured at each setting. These optical density measurements were made with an Optical Densitometer. Also, a scum cycle test was performed. In this test the fountain solution feed was momentarily stopped to allow the plate to become completely coated with ink. Then the fountain solution feed was started and the number of revolutions of the plate before it was cleaned of excess ink was recorded. Further, visual observations were made of the print to determine the appearance of tinting and banding.

The results are shown in Table I.

### Example 1

The following ingredients were mixed together to form a fountain solution:
14.17 g (0.5 ounce) gum arabic
14.17 g (0.5 ounce) phosphoric acid (a 5% solution in water)
3600 g (127.0 ounce) water
36.85 g (1.3 ounce) 2-ethyl-1 ,3-hexanediol, and
192.8 g (6.8 ounce) propylene glycol

The formulation yielded a 1 volume percent concentration of 2-ethyl-1,3-hexanediol and a 5 volume percent concentration of propylene glycol.

The solution was tested as described in Control A.

The results are shown in Table I.

### Example 2

The following ingredients were mixed together to form a fountain solution:
14.17 g (0.5 ounce) gum arabic
14.17 g (0.5 ounce) phosphoric acid (a 5% solution in water)
3600 g (127.0 ounce) water,
36.85 g (1.3 ounce) 2-ethyl-1,3-hexanediol, and
192.8 g (6.8 ounce) dipropylene glycol

The solution was tested as described in Control A.

The results are shown in Table I.

### Example 3

The following ingredients were mixed together to form a fountain solution:
14.17 g (0.5 ounce) gum arabic,
14.17 g (0.5 ounce) phosphoric acid (a 5% solution in water)
3600 g (127.0 ounce) water
36.85 g (1.3 ounce) 2-ethyl-1,3-hexanediol, and
192.8 g (6.8 ounce) diethylene glycol

The solution was tested as described in Control A.

The results are shown in Table I.

### Example 4

The following ingredients were mixed together to form a fountain solution:
14.17 g (0.5 ounce) gum arabic
14.17 g (0.5 ounce) phosphoric acid (a 5% solution in water)
3600 g (127.0 ounce) water
36.85 g (1.3 ounce) 2-ethyl-1,3-hexanediol, and
192.8 g (6.8 ounce) hexylene glycol

The solution was tested as described in Control A.

The results are shown in Table I.

The data in Table I show that generally higher optical density values are obtained when 2-ethyl-1,3-hexanediol is mixed with a glycol. Also, the scum cycle values are generally lower when 2-ethyl-1,3-hexanediol is mixed with a glycol, which means that the addition of the glycol improves the cleansing operation. Further, addition of glycol to 2-ethyl-1,3-hexanediol tends to reduce tinting and banding.

### Examples 5 to 9

In these Examples fountain solutions were prepared using 2-ethyl-1,3-hexanediol and propylene glycol where the concentration of propylene glycol was varied.

### Example 5

The following ingredients were mixed together to form a fountain solution:
14.17 g (0.5 ounce) gum arabic
14.17 g (0.5 ounce) phosphoric acid (a 5% solution in water)
3600 g (127.0 ounce) water
36.85 g (1.3 ounce) 2-ethyl-1,3-hexanediol, and
73.7 g (2.6 ounce) propylene glycol

The formulation yielded a 2 volume percent concentration of propylene glycol.

The formulations were used on the press described in Control A. These different inks were used: offset ink No. 205; heatset web offset ink No. 204; and an acrylic modified sheet offset ink similar to No. 205 (National Association Printing ink Manufacturers, August, 1974). The optical density was measured. Also, the scum cycle test was performed.

The results are shown in Table II.

### Example 6

Example 5 was exactly repeated except that 147.4 g (5.2 ounces) of propylene glycol were used. The formulation yielded a 4 volume percent concentration of the glycol.

The results are shown in Table II.

### Example 7

Example 5 was exactly repeated except that 221.1 g (7.8 ounces) of propylene glycol were used. The formulation yielded a 6 volume percent concentration of the glycol.

The results are shown in Table II.

### Example 8

Example 5 was exactly repeated except that 294.8 (10.4 ounces) of propylene glycol were used. The formulation yielded an 8 volume percent concentration of the glycol.

The results are shown in Table II.

### Example 9

Example 5 was exactly repeated except that 368.5 g (13.0 ounces) of propylene glycol were used. The formulation yielded a 10 volume percent concentration of the glycol.

The results are shown in Table II.

## Claims

1. An improved fountain solution suitable for use in a lithographic offset printing press which solution contains between 0.5 and about 10 percent by volume of a mixture of a polyol and/or glycol ether partially soluble in water and a polyol and/or glycol ether completely soluble in water.

2. A fountain solution as defined in claim 1 wherein the glycol which is partially soluble in water comprises 2-ethyl-1 ,3-hexanediol.

3. A fountain solution as defined in claims 1 or 2 wherein the glycol which is completely soluble in water is selected from one or more of propylene glycol, ethylene glycol, dipropylene glycol, diethylene glycol, hexylene glycol, triethylene glycol, tetraethylene glycol, tripropylene glycol and 1,5-pentanediol.

## Patentansprüche

1. Verbesserte Befeuchtungslösung, die zur Verwendung in einer Flachdruck-Offsetdruckpresse geeignet ist, welche Lösung zwischen 0,5 und etwa 10 Volumenprozent eines Gemisches aus einem in Wasser teilweise löslichen Polyol und/oder Glykolether und einem in Wasser vollständig löslichen Polyol und/oder Glykolether enthält.

2. Befeuchtungslösung, wie in Anspruch 1 definiert, worin das Glykol, das in Wasser teilweise löslich ist, 2-Ethyl-1,3-hexandiol enthält.

3. Befeuchtungslösung, wie in den Ansprüchen 1 oder 2 definiert, worin das Glykol, das in Wasser vollständig löslich ist, ausgewählt ist unter einem oder mehreren von Propylenglykol, Ethylenglykol, Dipropylenglykol, Diethylenglykol, Hexylenglykol, Triethylenglykol, Tetraethylenglykol, Tripropylenglykol und 1,5-Pentandiol.

## Revendications

1. Solution perfectionnée de mouillage apte à être utilisée dans une presse d'impression lithographique offset, cette solution contenant entre 0,5 et environ 10% en volume d'un mélange d'un polyol et/ou d'un éther de glycol partiellement soluble dans l'eau et d'un polyol et/ou d'un éther de glycol complètement soluble dans l'eau.

2. Solution de mouillage telle que définie dans la revendication 1, dans laquelle le glycol qui est partiellement soluble dans l'eau comprend du éthyl-1,3-hexanediol.

3. Solution de mouillage telle que définie dans les revendications 1 ou 2, dans laquelle le glycol qui est complètement soluble dans l'eau comprend un ou plusieurs glycols choisis entre le propylène- glycol, l'éthylèneglycol, le dipropylèneglycol, le diéthylèneglycol, l'hexylèneglycol, le triéthylèneglycol, le tétraéthylèneglycol, le tripropylèneglycol et le 1,5-pentanediol.
